



3

impurities in the inorganic metal salt from interfering with the brightening effect of the brightening additive.

The quantity of the S-alkanesulfonic acid compounds added to electroplating baths according to the present invention may range from 0.01 to 20 gm. per liter of bath. The effective current density range of such electroplating baths lies between 0.5 and 12 amp./dm.<sup>2</sup>, and the temperature of the solution may reach as high as 60° C. during the electroplating procedure. The current density range at which the optimum brightening effect is achieved will vary from one particular brightener to the other, but in general the range is of considerable breadth for the entire group of brighteners herein disclosed. The optimum current density range may, however, be broadened by employing a mixture of two or more members of the group.

Particularly noteworthy is the fact that the addition of the S-alkanesulfonic acid compounds described herein to electroplating baths makes it possible to produce full-bright electroplates within an exceptionally broad range of temperatures, namely between 15 and 60° C. At temperatures higher than room temperature the optimum current density range is shifted toward considerably higher values (about 15 amp./dm.<sup>2</sup>). Moreover, because of the ability of our brightening agents to produce full-bright electrodeposits at relatively high bath temperatures, it is possible to use the brighteners in copper-plating baths which because of high rates of current flow develop a considerable amount of heat and therefore operate at temperatures up to 40° C. and even 50° C.

Electroplating baths modified in accordance with our invention may be employed to deposit metal electro-deposits on any desired customary base metal, such as iron, steel, zinc and similar non-precious metals or alloys thereof. In the case of copper-plating baths, the base metal may first be provided with a thin copper coating in a separate cyanide bath in customary fashion, or the base metal may be provided directly with the final copper plate without a preliminary thin copper base coat in accordance with the process disclosed in copending application Serial No. 458,983, filed September 28, 1954.

In all cases, electroplating baths modified in accordance with the present invention produce full-bright electrodeposits of extraordinary high quality which do not require subsequent buffing or polishing.

The following examples will further illustrate the present invention and enable others skilled in the art to understand it more completely. It will be understood, however, that the invention is not limited to these particular examples.

*Example 1*

0.3 to 1.5 gm. per liter of the trisodium salt of 1,3,5-triazine-2,4,6-tri-(mercaptopropane-1-sulfonic acid) having the structural formula



were dissolved in an acid aqueous copper sulfate bath composed of water, 220 gm. per liter crystalline copper sulfate and 60 gm. per liter sulfuric acid. Sheet metal objects copper-plated in this electroplating solution at room temperature and at elevated temperatures up to 60° C. with a current density from 0.5 to 8 amp./dm.<sup>2</sup> were provided with a full-bright copper electrodeposit which did not require buffering or polishing.

### *Example II*

The same full-bright copper electrodeposits were obtained when 0.2 to 1.5 gm. per liter of the trisodium salt

4

of 1,3,5-triazine-2,4,6-tri-(mercaptopropane-2-hydroxy-1-sulfonic acid) having the structural formula



or the trisodium salt of 1,3,5-triazine-2,4,6-tri-(mercaptoethane-1-sulfonic acid) having the structural formula



20 were added to the acid copper sulfate solution described in Example I instead of the trisodium salt of 1,3,5-triazine-2,4,6-tri-(mercaptopropane - 1 - sulfonic acid), and brass and iron objects were copper-plated therein under the conditions of temperature and current density described in Example I.

### *Example III*

0.5 to 1.0 gm. per liter of the disodium salt of 1,3,4-thiodiazole-2,5-bis-(mercaptopropane - 1 - sulfonic acid) 30 having the structural formula



was added to an acid copper sulfate solution composed of water, 200 gm. per liter crystalline copper sulfate and 60 gm. per liter sulfuric acid. Brass and iron objects electroplated in this solution at current densities from 2 to 10 amp./dm.<sup>2</sup> and at temperatures between room temperature and 45° C. were provided with a full-bright, high-quality copper plate which required no buffering or polishing subsequent to rinsing.

#### *Example IV*

0.2 to 1.0 gm. per liter of the dipotassium salt of N,N'-methylene-di-(isothiourea-S - propane - 1 - sulfonic acid) having the structural formula



was added to the acid copper sulfate solution of Example III instead of the disodium salt of 1,3,4-thiodiazole-2,5-bis-(mercaptopropane-1-sulfonic acid). Brass and iron objects electroplated in this modified copper sulfate bath at current densities from 1 to 11 amp./dm.<sup>2</sup> and at temperatures between room temperature and about 50° C. were provided with full-bright, high-quality copper plates which required no buffing or polishing.

*Example V*

65 1.2 gm. per liter of the trisodium salt of 1,3,5-triazine-  
2,4,6-tri-(mercaptopropane-2-hydroxy - 1 - sulfonic acid)  
having the structural formula shown in Example II and  
0.8 to 1.2 gm. per liter 1,3-bis-(dibutylamino)-propanol-2,  
described in said copending application Serial No. 458,984,  
were added to an acid copper sulfate solution composed  
of water, 220 gm. per liter crystalline copper sulfate and  
60 gm. per liter sulfuric acid. Brass and iron objects  
70 electroplated in this solution at temperatures from room  
temperature to 60° C. and at current densities from  
slightly above 0 amp./dm.<sup>2</sup> up to 15 amp./dm.<sup>2</sup> were  
provided with full-bright copper electrodeposits of excep-  
75 tionally high quality which required no additional buffing  
or polishing.



gen, alkali metal and ammonium, and  $n$  is an integer equal to the number of said carbon atoms in the radical R, said brightening agent being present in sufficient amount to effect the brightening action.

6. The process according to claim 5, wherein R is a 5 1,3,5-triazine radical.

7. The process according to claim 5, wherein R is a 1,3,4-thiodiazole radical.

8. The process according to claim 5, wherein R is a 10 N,N'-methylene-di-isothiourea radical.

9. The electroplating bath of claim 1 wherein the quantity of brightener in said bath is between about 0.01 to 20 gm./liter.

10. The process of claim 5 wherein the quantity of brightener used is between about 0.01 to 20 gm./liter.

References Cited in the file of this patent

UNITED STATES PATENTS

10 2,647,866 Brown ----- Aug. 4, 1953

UNITED STATES PATENT OFFICE  
CERTIFICATE OF CORRECTION

Patent No. 2,849,352

August 26, 1958

Alfred Kirstahler et al.

It is hereby certified that error appears in the printed specification of the above numbered patent requiring correction and that the said Letters Patent should read as corrected below.

Column 2, lines 3 to 5, for that portion of the formula reading

$$\begin{array}{c} \text{OH} \\ | \\ \text{HO}_3\text{S}-\text{CH}_2-\text{CH}-\text{CH}_3-\text{S}-\text{C} \end{array}$$
 read -- 
$$\begin{array}{c} \text{OH} \\ | \\ \text{HO}_3\text{S}-\text{CH}_2-\text{CH}-\text{CH}_2-\text{S}-\text{C} \end{array}$$
 --; column 3, line 58, Example I, for that portion of the formula reading " $\text{NaO}_2\text{S}-$ " read --  $\text{NaO}_3\text{S}-$  --; column 4, line 14, Example II, for that portion of the formula reading " $\text{NaO}_3\text{SN}$ " read --  $\text{NaO}_3\text{S}-$  --.

Signed and sealed this 30th day of December 1958.

Attest:

KARL H. AXLINE  
Attesting Officer

ROBERT C. WATSON  
Commissioner of Patents